

Aug. 19, 1924.

1,505,323

G. B. EBERENZ

PROCESS OF CONCENTRATING ORES

Original Filed April 15, 1920



Inventor  
George B. Eberenz  
by Emil Staren Atty.

Patented Aug. 19, 1924.

1,505,323

# UNITED STATES PATENT OFFICE.

GEORGE B. EBERENZ, OF EL PASO, TEXAS, ASSIGNOR OF ONE-FOURTH TO EDWARD P. MATHEWSON, OF NEW YORK, N. Y., AND THREE-FOURTHS TO THOMAS J. SCANLON, OF ALTON, ILLINOIS.

## PROCESS OF CONCENTRATING ORES.

Application filed April 15, 1920, Serial No. 374,077. Renewed January 5, 1924.

To all whom it may concern:

Be it known that I, GEORGE B. EBERENZ, a citizen of the United States, residing at El Paso, in the county of El Paso and 5 State of Texas, have invented certain new and useful Improvements in Processes of Concentrating Ores, of which the following is a full, clear, and exact description, reference being had to the accompanying drawings, forming a part hereof.

The present invention is directed to improvements in processes of concentrating ores by flotation, the object sought being to produce a mineral froth floatable on the 15 surface of the pulp under treatment by subjecting the pulp to the action of sulfureted hydrogen gas or other reducing or non-oxygenous reagent while the pulp is undergoing agitation in a suitable container, without the use of selective agents 20 such as frothing oils or oily substances usually depended on to segregate the mineral components (mainly sulfids) from the non-mineral particles or gangue. To produce a 25 coherent froth carrying the mineral particles without resort to frothing oils, the reagent employed must be delivered to the pulp (except perhaps during the last stages of the operation) without access of atmospheric air in order to avoid possible oxidation 30 of any sulfid mineral particles, and to facilitate and ensure the desired reaction between the oxidized mineral particles and the active element (sulfur) of the reagent employed. While sulfureted hydrogen 35 ( $H_2S$ ) is the preferred reagent used under my process I do not wish to be restricted thereto, any soluble sulfid (particularly alkali sulfids) or carrier of sulfur acting in 40 an equivalent capacity falling within the spirit of my invention. The sulfureted hydrogen gas may either be injected into the pulp below the surface thereof, or the charge of pulp undergoing treatment may 45 be subjected to the action of the gas under pressure maintained in contact with the surface of the pulp while the latter is (preferably) mechanically agitated, the agitation being necessary to ensure a thorough impregnation and aeration of the pulp mass by the gas, or at least a sufficient impregnation and aeration to effect the frothing 50 which is needed to concentrate the mineral particles of the ore. By my process oxi-

dized ores such as carbonates, oxids, silicates and the like undergo sulfidation; and if any natural sulfids are present, these, together with the sulfidized particles will be carried into the froth at certain stages of the operation, the frothing being facilitated in the majority of cases, by keeping the pulp as nearly neutral as possible by means of lime, caustic alkali, or equivalent reagent, though a slight acidity with some ores is not harmful. In order to determine 65 how much sulfureted hydrogen shall be employed to produce an ideal mineral "gas" froth, the following observations as to oil flotation will be pertinent. In oil flotation air plays a very important part in the formation of the bubbles which result in the final froth. At the same time in what is today recognized as an ideal oil flotation process dependence is had on the presence 70 of a fraction of one per cent of oil (on the ore) which, as well understood in the art has a preferential affinity for the mineral particles when in the form of sulfids. This affinity is no doubt due to the reaction 75 between the sulfur of the minerals and the hydrogen of the oil resulting in the formation of sulfureted hydrogen which is recognized as a reducing agent, and as such it no doubt plays an important part in preventing oxidation of the mineral particles 80 by the air with which the pulp is charged and by which they are floated, oxidation of the mineral particles destroying or materially impairing the affinity which the oil 85 manifests therefor when the same are in the form of sulfids. By my process, in lieu 90 of forming the sulfureted hydrogen by the reaction above indicated (between the sulfur of the mineral sulfids and the hydrogen of the oil) I introduce this reagent into the pulp from an outside source, the quantity so introduced being governed by considerations of the same character as control the 95 quantity of oil employed in oil flotation, that is to say, where oxidized ores (with or without natural sulfids) are treated, only so much hydrogen sulfid need be used as will sulfidize at least superficially the oxidized particles of the minerals, any excess of the reagent being avoided in order not 100 to impart to the sulfidized particles too great a specific gravity or one unfavorable to the production of a coherent mineral 105

froth, it being understood that the sulfids of most of the metals are heavier than the oxids though having a greater affinity for the aerating gases than have the oxids. In 5 my process a certain degree of elasticity may be imparted to the froth by the addition to the pulp of a small quantity (a pinch) of rosin in powdered form, the presence of the rosin likewise assisting in the 10 frothing operation. It was pointed out above that except at the later stages of the process, the operation should be carried on without access of atmospheric air. In this 15 connection it may be stated that inert gases such as nitrogen, carbonic acid and the like are not only not deleterious but tend to assist the frothing presumably for the reason that they do not oxidize the mineral particles sulfidized by the sulfureted hydrogen. These inert gases may come from 20 the atmosphere, or, in the case of carbonic acid gas, this may be evolved from the mineral and other carbonates contained in a pulp to which a slight quantity of acid 25 (mineral acid) has been added to bring about neutralization of an alkaline pulp, or purposely added to slightly acidify a neutral pulp, it being understood that while I prefer to operate on a neutral pulp a 30 slight acidity or even alkalinity with some ores is not detrimental to the general results obtained by my invention. The instrumentalities employed in practicing my process are not important, any suitable flotation 35 machine capable of preserving the working conditions essential to the success of the process answering the purpose. In the drawings, I show one type of machine but other types may be used. The details of 40 the invention will now be described in connection with the accompanying drawings in which—

Figure 1 represents a side elevation of a 45 concentrating tank or cell suitable for carrying on my new process, parts being in section; Fig. 2 is a top plan of Fig. 1 with parts broken away; and Fig. 3 is a diagrammatic side elevation showing three cells in series.

Referring to the drawings, 1 represents 50 a suitable (preferably concrete) tank or cell provided with a stirring compartment  $\alpha$  and a froth compartment  $\beta$ , the two compartments being separated by a partition wall  $w$  provided with a slot or circulating opening  $o$  near the center thereof, said opening extending the width of the cell, a similar but narrower circulating opening  $o'$  being formed between the lower edge of the 55 partition wall and the bottom of the cell. The froth compartment is preferably provided with an inclined wall  $w'$  opposite the wall  $w$ , the said inclined wall being provided with a transverse overflow edge  $e$  60 depressed below the side walls of the cell,

the froth  $h$  flowing over said edge into a launder 2 from which the froth is conducted to any suitable point for further treatment. Leading from the inclined wall  $w'$  near the base thereof is a spout 3 which 70 discharges the tailings from the cell 1 into the stirring compartment  $\alpha'$  of a second cell 1', the vertical end wall of the latter being provided with a pulp inlet opening  $m'$  into which the spout 3 is inserted. The corresponding wall of the cell 1 is provided 75 with a pulp inlet  $m$  which may be coupled to any suitable source of pulp supply (not shown). Disposed transversely of the compartment  $\alpha$  below the circulating opening  $o$  is a stirrer or beater shaft 4, the same being provided inside said compartment  $\alpha$  with a series of radially disposed arms 5 to the outer ends of which are secured the perforated beaters or blades 6, the latter being 80 disposed parallel to the axis of the shaft as shown (Fig. 2). The outer edges of the blades are substantially opposite the center line of the opening  $o$  when they reach the highest point of their upward 85 sweep, and opposite the opening  $o'$  when at the lowest point of their downward sweep, this arrangement ensuring a thorough circulation of the beaten pulp through 90 said openings, it being understood that the beaters revolve toward the opening  $o'$  and from the opening  $o$  (counter-clockwise in Fig. 1). The top of each cell is provided 95 with a hinged or equivalent lid  $L$  which closes air-tight when clamped down. The aerating medium or sulfureted hydrogen gas is contained in a gas tank 7 from which leads a pipe 8 to the compartment  $\alpha$  through the top of the cell, a similar branch pipe 8' leading to the stirring compartment  $\alpha'$  of the cell 1', the pipes being provided 100 at convenient points with controlling needle valves  $V$  of any approved pattern known to the art, the quantities of gas admitted to the cells being carefully regulated by 105 said valves. In the example before us only two cells 1, 1', are shown but it is obvious that we may have a series of three (or more) cells 1, 1', 1'', any cell receiving the 110 tailings of the cell immediately preceding, and discharging its concentrates or mineral froth into its own launder as shown in the diagrammatic illustration in Fig. 3. The beater shaft 4 extends through the side walls of the cell being supported near the walls in bearings 9, the shaft extending 115 beyond one of the bearings and carrying a pulley  $P$  from which extends a belt  $B$  to a pulley  $P'$  of the shaft of a suitable electric motor  $M$ . Any other method of 120 driving the stirrer shaft may however be resorted to, and any suitable mechanical connections within the purview of the skilled mechanic may be employed to drive the stirrers of the remaining cells of the 125

series. Since all the cells and their mode of operation are the same, a description of one will suffice for all, and accordingly the description of the operation of the process 5 will be confined to the main or first cell 1 of the series. This operation is substantially as follows:

Pulp is fed to the compartment *a* through the inlet *m* by a nozzle or pipe *A* leading 10 from any suitable source of pulp supply (not shown), the lid *L* being clamped down so as to exclude the air, thereby promoting sulfidation and minimizing the danger of oxidation of the mineral particles sulfidized 15 by the sulfureted hydrogen (assuming that we are treating oxidized ores) admitted into the cell. At the same time, by a proper control of the valve *V*, suitable quantities of sulfureted hydrogen under pressure are admitted 20 into the compartment *a*, the beater or stirrer shaft having in the meantime been set into motion so that the pulp contents of the cell are not only beaten, but during the beating operation the gas above 25 the pulp being under pressure, impregnates the molecules of the beaten pulp, the mechanical agitation of the pulp assisting in effecting a thorough mixing thereof with, and aeration by, the gas, the bubbles resulting 30 from the combination of operations rising through the liquid pulp in the compartment *b* where the portions of the pulp above the plane of the opening *o* are comparatively quiescent, the froth *h*, being a 35 mineral froth (in contradistinction to an oil froth), floating on the surface of the pulp in the froth compartment *b* and flowing over the edge *e* into the launder 2. The beating or stirring of the pulp in the compartment *a* causes the liquid to circulate 40 between the compartments *a*, *b*, substantially as indicated by the arrows in Fig. 1, and as more pulp is added to the charge more froth is formed and carried away 45 by the launder 2. The tailings from cell 1 are constantly discharging through the spout 3 into the next cell where the same are subjected to like treatment. These tailings not only include sands or gangue having 50 no value, but considerable mineral matter which has escaped treatment in the first cell. After the pulp has traversed a number of cells, the tailings from the last cell are discarded containing as they do only 55 the gangue with perhaps a negligible amount of mineral. Obviously, and especially for the reason that the sulfureted hydrogen is under pressure, the level of the liquid in the cell must be kept above the inlet *m*; 60 otherwise the gas would escape from the cell. It is even possible that the level of the pulp in the compartment *a* may be depressed below that in the compartment *b*, by the pneumatic pressure of the gas above 65 the liquid in the compartment *a*; but ob-

viously the depression should not be carried below the plane of the lower end of the inlet *m*. The inlet may of course be dropped below the position shown in the drawing should it be desirable to use gas 70 under a high pressure. During the later stages of the operation the sulfureted hydrogen may be discontinued, the lid *L* raised, and air admitted to the pulp while being stirred, the air serving to arrest any tendency to oversulfidation of any given charge of ore operated on, especially in cases where natural mineral sulfids are associated with the oxidized ores (carbonates, oxids, silicates) undergoing sulfidation for purposes of making froth. The gas may be cut off at the tank 7 by means of an ordinary globe valve *V'* well understood in the art. The precise chemical reactions which take place in the cell need not be gone into because varying with different charges of pulp, but in a general way it may be stated that in treating what are known as oxidized ores (as distinguished from sulfids) these are sulfidized by the sulfureted hydrogen to the extent necessary to form an outer coat of sulfid on the larger mineral particles (the ore being ground to the usual degree of fineness as practiced in the flotation art), 85 the smallest particles being possibly sulfidized all the way to the center. The prevailing ores treated are oxidized ores of copper, zinc, and lead, though chlorid of silver may likewise be successfully floated by my process. The bases of any metallic salts that may be held in solution by the pulp waters may likewise be sulfidized (usually in the form of precipitates of the sulfids of the metals) and floated with the main bulk of sulfidized particles derived 90 from the oxidized mineral particles held in suspension in the pulp water. In all cases oversulfidation, or sulfidation to or beyond the point of saturation should be avoided, as the formation of saturated sulfids in many cases increases the specific gravity of the mineral particles as compared with their specific gravity in the oxidized or semi-oxidized and sulfidized state, and hence 95 renders them less susceptible to flotation than in those cases where the sulfidation is arrested at a point where the specific gravity of the mineral particle is still comparatively low. Of course the point to which the sulfidation shall be carried depends on the ore treated, and every new ore should first be tested in this regard. In the majority of cases the mineral froth formed by the sulfureted hydrogen is sufficiently coherent to 100 maintain its integrity while being floated to and out of the froth launder 2, but should it be desirable to render the froth more elastic, a pinch of rosin may be added to the pulp in the cell during the beating or stirring operation. The stirrer blades con-

stantly churn the contents of the cell, and thereby cause different particles of the pulp to present themselves to the superincumbent body of gas in the compartment *a* until the 5 entire liquid body is impregnated with the gas which upon its release in the compartment *b* rises to the surface in bubble form taking with it the sulfidized mineral particles in the form of a coherent mineral 10 froth. The process is likewise applicable to sulfid ores but obviously the amount of sulfureted hydrogen used would be materially reduced as compared with that employed in connection with oxidized ores 15 that must first be sulfidized before they will attach themselves to the bubbles formed by the gas with which the pulp is charged.

Having described my invention what I claim is—

20 In the concentration of ores, the process which consists in subjecting a charge of ore

in pulp form while under agitation to the action of sulfureted hydrogen maintained under pressure against the pulp mass to the exclusion of other selective agents and out 25 of contact with the atmosphere to sulfidize the mineral particles and aerate the pulp mass, then cutting off the supply of hydrogen sulfid, and continuing the agitation in contact with the air at normal atmospheric 30 pressure, causing the resulting bubbles and mineral particles adhering thereto to migrate through the pulp to a region of comparative quiet, and removing the resulting froth from the surface of said region. 35

In testimony whereof I affix my signature, in presence of two witnesses.

GEORGE B. EBERENZ.

Witnesses:

J. A. CAMEL,  
ELLA O'HARA.